

May 3, 1966

F. J. STARK, JR., ET AL

3,249,525

WAX REFINING

Filed Feb. 9, 1961



1

3,249,525  
WAX REFINING

Fred J. Stark, Jr., Kirkwood, and Robert M. Thompson, Clayton, Mo., assignors to Petrolite Corporation, Wilmington, Del., a corporation of Delaware  
Filed Feb. 9, 1961, Ser. No. 88,216  
6 Claims. (Cl. 208—27)

This invention relates to an improved process for refining hydrocarbon waxes. More particularly, this invention relates to an improved wax refining process whereby petroleum wax is improved by the removal of, or by the reduction in, color and color-forming bodies, aromatic content, sulfur, nitrogen, combined oxygen, trace metals and other undesirable materials present in the wax. This invention also relates to the products produced by the process, and particularly to a hydrocarbon wax characterized by substantial freedom from aromaticity.

In refining hydrocarbon waxes, such as those derived from petroleum, it is necessary to purify the product so as to remove color and other undesirable impurities. It is generally difficult to produce white wax since complete removal of color bodies from wax is quite difficult. In addition, it is desirable to remove certain undesirable materials which exist in trace quantities.

Recently there have been additional standards imposed on waxes which come in contact with food whereby restrictions have been placed on the presence in waxes of certain compounds containing aromatic condensed ring systems, i.e. compounds where one aromatic ring is fused to at least one other aromatic ring so as to retain general aromaticity, such as in anthracene, phenanthrene, pyrene, benanzthracene, dibenzanthracene, benzpyrene, etc.

We have now discovered a process for refining hydrocarbon waxes whereby such waxes are improved by the removal of, or by the reduction in, color and color-forming bodies, aromatic content, sulfur, nitrogen, combined oxygen, trace metal content and other undesirable materials present in wax. Our process is particularly effective in removing or reducing the presence of compounds containing aromatic condensed ring systems, also referred to herein as "condensed ring aromaticity."

The waxes refined according to this invention are hydrocarbon waxes, such as petroleum waxes. These include (1) tank bottom derived microcrystalline wax; (2) residual lube stock derived microcrystalline wax; (3) intermediate lube stock derived wax; and (4) paraffin wax.

The figure of the hereinafter cited Bruce Clary article presents an excellent schematic outline for preparing these waxes. The waxes themselves, or products intermediate in the preparation of these waxes, can be treated in the manner of this invention. For convenience, a number has been assigned to designate each wax type and intermediate formed during the processes. The number indicates the product formed upon completion of the indicated process step in the general line of prior process steps. For example, 8 (first vertical column of blocks, block "Deoiling") is the product formed after the deoiling of deasphalted, distillation residue from dehydrated crude tank bottoms; 15 (second vertical column of blocks, block "Deoiling") is the product formed after the deoiling of deasphalted, dewaxed residual lube stocks. Certain non-limiting wax intermediates presented in Table I, will be employed in the examples to illustrate the invention.

2

TABLE I

|    | Wax No. (Fig. 1)                                                                                                                  | Type of Wax                                                                                       |
|----|-----------------------------------------------------------------------------------------------------------------------------------|---------------------------------------------------------------------------------------------------|
| 5  | 8 (block "Deoiling," first vertical column of blocks).                                                                            | Crude Tank Bottom derived microcrystalline wax subsequent to deoiling.                            |
|    | 14 (block "Petroletum," second vertical column of blocks).                                                                        | Petroletum.                                                                                       |
| 10 | 15 (block "Deoiling," second vertical column of blocks).<br>20 (block "Crude Intermediate Wax," third vertical column of blocks). | Crude Residual microcrystalline wax after deoiling.<br>Crude Intermediate wax prior to deoiling.  |
|    | 21 (block "Deoiling," third vertical column of blocks).<br>27 (block "Solvent Deoiling," fourth vertical column of blocks).       | Crude Intermediate wax subsequent to deoiling.<br>Crude Scale wax subsequent to solvent deoiling. |

Our process can be used as a substitute for the decolorization processes now employed in the manufacture of tank bottom, microcrystalline, residual microcrystalline, intermediate wax and refined paraffin, for example, in place of contacting the wax with an absorbent material such as bauxite, clay, alumina, silica gel, charcoal and the like.

Petroleum waxes and the processes by which they are manufactured are too well known to require further elaboration. In this regard note the following publications:

- (1) "How to Judge, Use and Handle Microcrystalline Waxes" by Bruce Clary, "Paper, Film & Foil Converter," September and October, 1955.
- (2) The Chemistry and Technology of Waxes by Warth, published by Reinhold, 2d edition (1956).
- (3) "Decolorization of Petroleum Waxes by Absorbent Percolation" by Willis A. Johnston, "Petroleum Processing," pages 2-8, September 1947.
- (4) Commercial Waxes, by H. Bennet, Chemical Publishing, 2d edition (1956).

An excellent schematic presentation of the steps employed in the manufacture of petroleum wax can be found in FIG. 1 of the Bruce Clary article (1), which is referred to here in column 1, and particularly in Table I above.

Our refining processes are outlined schematically in the figure.

*A process.*—The wax to be refined I is treated with an alkali metal (with or without ether) to yield wax and precipitate II. This product is then treated with CO<sub>2</sub> and the precipitate removed to yield wax AI. Wax AI can be further refined by hydrogenation, followed by precipitate removal, to yield refined wax AII.

*B process.*—The wax to be refined I is treated with an alkali metal (with or without ether) to yield wax and precipitate II. This product is then treated with oxygen and the precipitate removed to yield wax BI. Wax BI can be further refined by hydrogenation, followed by precipitate removal to yield refined wax BII.

*C processes.*—The wax to be refined I is treated with alkali metal (with or without ether) to yield wax and precipitate II. The precipitate is then removed to yield wax filtrate III which (if it tests positively for condensed ring aromaticity) is then treated with alkali metal, preferably with ether, at point H, then treated with CO<sub>2</sub>, followed by precipitate removal, to yield wax CI. Wax CI can be further refined by hydrogenation, followed by precipitate removal to yield refined wax CII.

*D process.*—The wax to be refined I is treated with alkali metal (with or without ether) to yield wax and

precipitate II. The precipitate is then removed to form wax filtrate III which (if it tests positively for condensed ring aromaticity) is then treated with alkali metal, preferably with ether, at point I, followed by treatment with O<sub>2</sub> and precipitate removal to yield wax DI. Wax DI can be further refined by hydrogenation followed by precipitate removal to yield refined wax DII.

*E process.*—The wax to be refined I is treated with alkali metal (with or without ether) to yield wax and precipitate II and the precipitate removed to yield wax 10 filtrate III which is then hydrogenated, followed by precipitate removal, to yield refined wax EI. If hydrogenation is carried out with an active hydrogen compound (instead of hydrogen), alkali metal, preferably with ether, is added at point J.

*F process.*—The wax to be refined I is treated with alkali metal (with or without ether) to yield wax and precipitate II which is then hydrogenated and the precipitate removed to yield refined wax (FI). Since the presence of the precipitate tends to shorten the life of the hydrogenation catalyst, this hydrogenation is carried out with an active hydrogen compound rather than with hydrogen.

Although alkali metals alone, with or without ether, or these alkali metal treated products further treated with CO<sub>2</sub> or O<sub>2</sub>, with or without ether, produce refined waxes, 25 these waxes can be further refined according to these processes in combination with hydrogenation.

In the above processes subsequent to reaction with alkali metal employing ether, ether is removed by any suitable means, for example, by distillation prior to removal of the 30 precipitate. This reduces the solubility of the precipitate in the wax.

The product of any sequence of steps can be rerun according to the very same process employing all of the same sequence of steps, or less than the full sequence of steps; or the product of any sequence of steps can be rerun according to another sequence of steps, or less than the full sequence of steps, of any process outlined in the figure. For example, the product AII can be rerun according to the same process which has produced AII, 35 or the product of AII can be rerun by the A process up to AI, or the product BII can be rerun according to the C process, or product CII can be rerun according to D process, etc.

It is noted in the figure that the wax to be refined can be treated with alkali metal with or without ether at point G. Although both methods can be employed, in the preferred embodiment we first treat with an alkali metal in the absence of ether. This procedure tends to yield a lighter wax having a lower sulfur content than is produced by treatment with alkali metal in the presence of ether. On the other hand, the use of alkali metal in the presence of ether facilitates the alkali metal reaction.

Therefore, it is preferable that the initial alkali metal treatment be carried out without ether and the wax and precipitate II thus obtained be filtered to yield wax filtrate III. Wax filtrate III can be hydrogenated with hydrogen to yield refined wax EI. This preferred procedure is outlined as follows:

Preferred E process—



Where it is desired to carbonate, to oxygenate, or to treat with an active hydrogen compound wax filtrate III, which has been treated with alkali metal without ether, it is preferable to treat said wax filtrate III with alkali metal with ether prior to oxygenation, carbonation, or treatment with an active hydrogen compound.

In general, the chief reason for hydrogenating, oxygenating and carbonating is to remove or reduce condensed ring aromaticity still present in the wax after alkali metal treatment. Therefore, after filtration of the alkali metal-treated wax it is advisable to examine the wax filtrate for condensed ring aromaticity. If the wax filtrate tests positively for condensed ring aromaticity, one adds additional alkali metal, preferably with ether, at points H, I and J, and then proceeds to carbonate by C process, or oxygenate by D process, or treat with an active hydrogen compound by E process. It should be noted that this alkali metal addition is made only if hydrogenation is carried out employing a compound containing an active hydrogen. Additional alkali metal is not required if hydrogenation is carried out with hydrogen (H<sub>2</sub>).

It is to be noted that the most effective agent in removing condensed ring aromaticity in waxes by alkali metal treatment is the sodium-potassium alloy, for example the 50:50 Na:K alloy.

In the case of F process involving wax and precipitate II it is desirable that hydrogenation be carried out with a compound containing an active hydrogen rather than with hydrogen (H<sub>2</sub>) since the presence of the precipitate tends to shorten the life of the hydrogenation catalyst.

ALKALI METAL TREATMENT

In general, the process is carried out by treating the hydrocarbon wax with an alkali metal, for example Li, Na, K, Ru, etc., and alloys thereof. For convenience and intimacy of contact, this treatment is carried out while the wax is in a liquid state. This liquid state can be achieved by heat, solution or a combination of both. Since the process is sensitive to many solvents, when it is desirable to employ a solvent, it should be a non-reactive liquid hydrocarbon in which the wax is soluble. Because of the reactive nature of alkali metals it is highly desirable to carry out this reaction in a dry, inert atmosphere such as in the presence of a solvent having a high vapor pressure, a dry inert gas such as nitrogen, etc.

Although the reaction may be carried out over a broad temperature range, the reaction in general is carried out from about the melting point of the wax up to below its decomposition temperature. In practice, the reaction is carried out at a temperature above about 60°, such as 60° to 300°, for example 100° to 275°, but preferably 200° to 250°. The time of the reaction will vary depending on other reaction conditions. In general, reaction time can vary from at least five minutes, such as 5 to 600 minutes, for example 10-200 minutes, but preferably 15 to 120 minutes.

When the alkali metal is mixed with wax, a black precipitate is formed. This precipitate is removed by any suitable means, for example, by centrifugation, filtration, solvent extraction, for example by using liquid propane, 55 adsorption on an active surface, etc. Removal of the precipitate yields a wax which is not only light in color but also contains less sulfur, nitrogen, combined oxygen, trace metals, aromatics and other undesirable materials.

Although the nature of the reaction taking place during the process is not understood, it is believed, among other things, that the reaction takes place between the alkali metal and petroleum resins, asphaltenes, aromatics, sulfur and nitrogen containing materials and other undesirable impurities present in the wax.

The alkali metal is employed in amounts sufficient to decolorize the wax, for example, in at least about 0.005% by weight of alkali metal based on the wax or crude wax charge, such as 0.01 to 10.0% or higher, for example 0.01 to 2.0%, but preferably 0.02 to 1.0%.

ALKALI METAL-ETHER TREATMENT

Although the alkali metal treatment can be run without a solvent, it can also be carried out in the presence of various inert solvents, for example, non-reactive hydrocarbons in which the wax is soluble. However, there is

a specific class of solvents which facilitates reaction so that reaction takes place within a shorter time under milder conditions. The action of the ether is specific, but it is not known whether the action is catalytic, whether the ether itself takes part in the reaction in some manner, or whether there are some solubility or other factors involved.

In practice, the temperature at which the reaction is run will depend on such factors as the solubility of the ether in the wax at the particular temperature, the boiling point of the ether, etc. Because many ethers are low boiling and do not dissolve wax at low temperatures, it is often desirable to run the reaction under super-atmospheric pressure so as to heat the reaction mixture to a temperature at which the ether dissolves the wax. Whenever the ether boils at a satisfactory range for example 75-200° C., it is convenient to run the reaction at the reflux temperature of the ether.

Suitable ethers include (1) aliphatic ethers containing a  $\text{CH}_3\text{O}$ -group and (2) cyclic aliphatic ethers, in each case the number of oxygen atoms and the number of carbon atoms being in a ratio of not less than 1:4. In the phrase "oxygen-carbon ratio of not less than 1:4" the ratio of 1:4 refers to the ratio of the number of oxygen atoms to the number of carbon atoms present in the ether. Examples of these ethers include the following:

Monoethers:



wherein  $n=1-3$ , for example



Polyethers:

Polyethers, for example, of polyhydric alcohols such as methylene glycols or others with more than one hydroxy group on the same carbon atom, e.g. ethyl orthoformate, methylal and other acetals; ketals; alkylene glycol ethers; etc., can be employed. These ethers may be expressed by the general formula:



where R is hydrogen or a lower alkyl group which R's may be the same or different provided that the ratio of oxygen to carbon is not less than 1:4, for example, the dimethyl ether of ethylene glycol, methyl ethyl ether of ethylene glycol, methyl propyl ether of ethylene glycol, corresponding propylene glycol ethers, trimethylene glycol ethers, etc.; polyethers of the general formula



where  $n$  and  $x$  are integers, for example 1-4 and at least one of the  $\text{C}_n\text{H}_{2n+1}$  groups is methyl, provided the ratio of oxygen to carbon is not less than 1:4, for example, the trimethyl ether, the dimethyl ethyl ether, the methyl diethyl ether, dimethyl isopropyl ether of glycerol, etc.

Other examples include the ethers of pentaerythritol, etc., having a  $\text{CH}_3\text{O}$ -group and a O/C ratio of not less than 1:4.

Suitable cyclic ethers include, for example, tetrahydrofuran, dioxolane, methyl glycerol formal, dioxane, etc.

Other suitable ethers include those of the general formula



where  $n=1-4$  and  $x=2-4$  with the proviso that the oxygen to carbon ratio is not less than 1:4, for example

the ethers of polyethylene glycols such as dimethyl ethylene glycol, dimethyl diethylene glycol, dimethyl dipropylene glycol, ethers of mixed alkylene glycol, for example



Other ethers not within the scope of the above, such as diethyl ether, diisopropyl ether, methyl phenyl ether, methyl benzyl ether, etc. may be reactive with certain more active alkali metals. In general, the ease with which the reaction starts decreases with increasing weight of the alkyl ether group. With methyl ethers of the higher alkyls, it may be necessary to add a small amount of an effective ether to start the reaction, as the reaction appears to be definitely autocatalytic when once started.

Within the restrictions above given as to the limitations of the ethers effecting the reaction, these ethers must furthermore not be split by the alkali metal under the conditions used. This does not mean that the ethers may not react in some way in some reversible reaction with the alkali metal since indications are that the ethers in effecting the reactions may, to some extent, take part in the reaction, but the ether must not be broken up or form irreversible reaction products. Thus, for example, ethylene oxide may be considered a cyclic ether falling within the limitations given for oxygen-carbon ratio; however, it reacts with the alkali metal and hence cannot satisfactorily perform the function required. There may be very slow ether cleavage with some good solvents, but at a rate much slower than that of the desired reaction. In order to simplify the wording later we further specify such ethers as are effective within our invention as being "stable" although as noted they may play some reactive role in causing the reactions to proceed.

The weight ratio of ether to wax can vary wide, for example, from at least about 1:25, or less, such as 1:25 to 25:1 or more, for example 1:4 to 4:1, but preferably 1:2 to 1:1.

However, the optimum amount present depends, among other factors, on the particular ether employed, the solubility of wax in the ether, etc.

To minimize solubility of the precipitate in the wax, ether is preferably removed prior to removal of the precipitate. This is conveniently done by distilling ether from the wax.

#### CARBONATION

After alkali metal or ether-alkali metal treatment, the reaction mixture can be carbonated by adding carbon dioxide thereto at any convenient temperature. Since the carbonation reaction does not appear to be temperature dependent but operative over a wide temperature range, all that is required is that the wax be in a liquid state. Thus, provided this state is maintained, carbon dioxide can be added in a gaseous state or added as solid Dry Ice. Super-atmospheric pressure may be employed to prevent carbon dioxide escape. If desired, the alkali metal treated wax can be added to an inert liquid medium containing carbon dioxide such as ethers, non-reactive hydrocarbons, etc.

In practice, the reaction is carried out at a temperature of at least 30° C. such as 30° to 200° C., for example 60° to 140 C., but preferably 80° to 100° C. The reaction is substantially instantaneous. In practice, we run the reaction for a period of at least five minutes, such as 5 to 120 min., for example 10 to 90 min., but preferably 15 to 60 min.

After carbonation of these waxes, the product is treated by any suitable means such as filtration, centrifugation, extraction, adsorption, etc., to remove insoluble materials.

In general, at least one gram-mol of carbon dioxide is added for each gram-atom of alkali metal added.

In practice excesses of carbon dioxide are employed by bubbling  $\text{CO}_2$  in the reaction mixture or adding solid

Dry Ice thereto. Where ether is employed, it is preferred to have the ether present during carbonation. Ether removal is effected after carbonation and prior to precipitate removal.

#### OXYGENATION

The alkali metal treated wax, or the ether-alkali metal treated wax, can also be treated with oxygen, an oxygen-containing gas such as air, ozone, etc. The process is carried out in the manner described for the carbonation process and under the same reaction conditions. Subsequent to oxygen addition any precipitate present is separated from the wax.

In general, at least one gram-mole of oxygen is added per gram-atom of alkali metal added. In practice, excesses of oxygen are employed by bubbling oxygen or an oxygen-containing gas, such as air, into the reaction mixtures.

As previously mentioned herein, the wax filtrate resulting from filtration of the alkali metal treated wax is tested for condensed ring aromaticity. If it tests positively for condensed ring aromaticity, additional alkali metal, preferably with ether, is added prior to carbonation or oxygenation. Where ether is employed, it is preferred to have ether present during oxygenation. Ether removal is effected after oxygenation and prior to precipitate removal.

microwax after deoiling (wax type 15) is employed under the conditions stated in Table II, Example 2.

#### Example 3

5 The process of Example 1 is repeated except that the wax product in Part I is extracted from the precipitate with liquid propane, and the wax product thereupon is freed of propane. The conditions employed are stated in Table II, Example 3.

10

#### Example 4

Petrolatum (100 g.) (wax No. 14) is treated with a lump of sodium (1 g.) in the manner of Example 1.

The precipitate in Part I is separated from the wax by means of a heated centrifuge. The conditions employed are stated in Table II, Example 4.

Since the following examples are carried out in a similar manner to save space, they will be presented in tabular form. The type of wax employed is identified by the numbers shown, which refer to the waxes of Table I. The wax products are blown with  $\text{CO}_2$  and  $\text{O}_2$  by passing these gases into the reaction mixture for ten minutes at the rate of about 1 g./min.

Where the products of Part I are further hydrogenated with a compound containing an active hydrogen (see 25 Table VI), some of unfiltered Part I product is preserved for such hydrogenation.

TABLE II.—ALKALI METAL TREATMENT

| Ex. | Wax Type | Alkali Metal     |                             | Temp. | Time in Hrs. | Method of Separation | Part I                                       | Part II | Part III |  |  |  |
|-----|----------|------------------|-----------------------------|-------|--------------|----------------------|----------------------------------------------|---------|----------|--|--|--|
|     |          | Name             | Weight Percent Metal in Wax |       |              |                      | Alkali Metal Plus Carbonylation (Unfiltered) | Temp.   | Temp.    |  |  |  |
|     |          |                  |                             |       |              |                      |                                              |         |          |  |  |  |
| 1   | 8        | Na               | 1.0                         | 250°  | 1            | Filtration           |                                              | 100     | 100      |  |  |  |
| 2   | 15       | Na               | 1.0                         | 200°  | 1            | do                   |                                              | 100     | 100      |  |  |  |
| 3   | 8        | Na               | 1.0                         | 250°  | 1            | Propane Extraction   |                                              | 150     | 125      |  |  |  |
| 4   | 14       | Na               | 1.0                         | 250°  | 1            | Centrifugation       |                                              | 100     | 100      |  |  |  |
| 5   | 15       | Na-K 50:50 alloy | 1.0                         | 175°  | 3            | Filtration           |                                              | 100     | 150      |  |  |  |
| 6   | 8        | Na               | 2.0                         | 200°  | 3            | do                   |                                              | 100     | 100      |  |  |  |
| 7   | 8        | Li               | 5.0                         | 150°  | 5            | Centrifugation       |                                              | 100     | 100      |  |  |  |
| 8   | 14       | Na               | 2.0                         | 190°  | 3            | do                   |                                              | 150     | 125      |  |  |  |
| 9   | 20       | Na               | 0.5                         | 200°  | 2            | Filtration           |                                              | 150     | 150      |  |  |  |
| 10  | 21       | Na               | 0.1                         | 200°  | 3            | do                   |                                              | 150     | 100      |  |  |  |
| 11  | 21       | K                | 0.1                         | 200°  | 2            | Propane Extraction   |                                              | 80      | 100      |  |  |  |
| 12  | 8        | K                | 0.05                        | 200°  | 1            | Filtration           |                                              | 80      | 100      |  |  |  |
| 13  | 27       | Na               | 0.05                        | 200°  | 0.5          | do                   |                                              | 150     | 80       |  |  |  |
| 14  | 27       | Na               | 1.0                         | 240°  | 1            | Centrifugation       |                                              | 100     | 80       |  |  |  |
| 15  | 8        | Na               | 0.02                        | 220°  | 1            | do                   |                                              | 150     | 75       |  |  |  |
| 16  | 8        | Na               | 0.05                        | 200°  | 1            | Filtration           |                                              | 75      | 100      |  |  |  |
| 17  | 8        | Na               | 0.1                         | 200°  | 1            | do                   |                                              | 100     | 100      |  |  |  |
| 18  | 15       | Na               | 0.1                         | 200°  | 1            | do                   |                                              | 100     | 100      |  |  |  |
| 19  | 15       | Na               | 0.05                        | 200°  | 0.5          | do                   |                                              | 150     | 150      |  |  |  |
| 20  | 14       | Na               | 0.05                        | 240°  | 0.5          | Propane Extraction   |                                              | 125     | 125      |  |  |  |
| 21  | 20       | Na               | 0.05                        | 200°  | 0.5          | Filtration           |                                              | 150     | 100      |  |  |  |
| 22  | 27       | K                | 0.05                        | 200°  | 0.5          | do                   |                                              | 200     | 150      |  |  |  |

TABLE II EXAMPLES

55

#### Example 1

Employing an inert atmosphere of dry nitrogen crude tank bottom derived microcrystalline wax after deoiling (100 g.) (wax type 8) and a lump of sodium (1 g.) are added to a dispersator. The temperature is raised to 250° C. while the dispersator is run at high speed for one hour to convert sodium to a fine dispersion. The temperature is maintained at 250° for about one hour. The product is then divided into three equal parts. In Part I the precipitate formed is then separated by filtration to produce a white wax which is essentially free of sulfur, nitrogen and oxygen. Part II (unfiltered) is blown with an excess of  $\text{CO}_2$  at 100° C. for ten minutes. The precipitate formed is then removed by filtration. Part III (unfiltered) is blown with an excess of  $\text{O}_2$  at 100° C. for ten minutes and the precipitate is separated by filtration.

#### Example 2

The above example is repeated except that crude residual

TABLE III EXAMPLES

#### Example 1

Type 8 crude wax (100 g.), 100 g. of 1,2-dimethoxyethane, and 0.1 g. of sodium are charged to a flask equipped with a stirrer and condenser. The reaction mixture is blanketed with dry nitrogen, heated to reflux and thus maintained for one hour. The product is then divided into three equal parts. In Part I, after removal of the ether by distillation, the precipitate formed is separated by filtration. Part II is blown with excess  $\text{CO}_2$  just above the melting point of the wax product for ten minutes. Then after removal of the remaining ether by distillation, the precipitate formed is separated from the wax by filtration. Part III is blown with an excess of  $\text{O}_2$  just above the melting point of the wax product for ten minutes, the remaining ether is removed by distillation and the precipitate formed is separated by filtration.

#### Example 2

The process of Example 1 is repeated except that tetrahydrofuran is employed in the amounts stated in Table III.

## Example 3

The process of Example 1 is repeated except that type

Table II), some of unfiltered Part I is preserved for such hydrogenation.

TABLE III.—ETHER-ALKALI METAL TREATMENT

| Ex. | Wax Type | Alkali Metal      |                             | Ether  |                           | Time, Hours | Part I Separation of Precipitate | Part II                                       | Part III                                     |
|-----|----------|-------------------|-----------------------------|--------|---------------------------|-------------|----------------------------------|-----------------------------------------------|----------------------------------------------|
|     |          | Name              | Weight percent Metal in Wax | Number | Weight Ratio Ether to Wax |             |                                  |                                               |                                              |
| 1   | 8        | Na                | 0.1                         | 1      | 1                         | 1           | Filtration                       | All examples are treated with $\text{CO}_2$ . | All examples are treated with $\text{O}_2$ . |
| 2   | 8        | Na                | 0.1                         | 2      | 0.5                       | 1           | do                               |                                               |                                              |
| 3   | 15       | Na                | 0.05                        | 4      | 1                         | 2           | do                               |                                               |                                              |
| 4   | 15       | Na                | 0.1                         | 3      | 1                         | 1           | do                               |                                               |                                              |
| 5   | 8        | Li                | 0.1                         | 1      | 1                         | 1           | do                               |                                               |                                              |
| 6   | 14       | K                 | 0.2                         | 1      | 0.5                       | 1           | do                               |                                               |                                              |
| 7   | 8        | Na-K 50:50 alloy. | 0.1                         | 2      | 0.25                      | 0.5         | Centrifugation                   |                                               |                                              |
| 8   | 8        | K                 | 0.5                         | 2      | 0.5                       | 0.5         | Propane Extraction               |                                               |                                              |
| 9   | 20       | Na                | 1.0                         | 4      | 0.25                      | 1           | Filtration                       |                                               |                                              |
| 10  | 21       | Na                | 2.0                         | 1      | 0.5                       | 1           | do                               |                                               |                                              |
| 11  | 27       | Na                | 0.05                        | 1      | 0.5                       | 1           | do                               |                                               |                                              |
| 12  | 27       | Na                | 0.1                         | 2      | 0.25                      | 1           | Centrifugation                   |                                               |                                              |
| 13  | 8        | Na                | 0.01                        | 2      | 0.75                      | 0.5         | Filtration                       |                                               |                                              |
| 14  | 15       | Na                | 0.01                        | 2      | 1                         | 1           | do                               |                                               |                                              |

15 wax and the dimethyl ether of diethyleneglycol are employed in the amounts stated in Table III.

## Example 4

Type 15 crude wax (100 g.), 100 g. of methyl isopropyl ether and 0.1 g. of sodium are charged to a rocker autoclave. The reaction mixture is heated to 90–100° C. and thus maintained for one hour under ambient pressure. This product is divided in three equal parts and treated in the manner of Example 1. The wax is raised to its melting point at which time the respective gases are added under pressure. Excess ether is removed during filtration.

Since the following examples are carried out in a similar manner, to save space, they will be presented in tabular form. The type of wax employed is identified by the number shown, which refers to the waxes of Table I. All reactions are run at reflux, employing one of the following ethers, except where methyl isopropyl ether is employed where the reaction is run at 90–100° C. in a rocker autoclave at ambient pressure.  $\text{CO}_2$  and  $\text{O}_2$  are added just above the melting point of the wax products.

- (1) 1,2-dimethoxyethane (B.P. 85.2° C.)
- (2) Tetrahydrofuran (B.P. 66° C.)
- (3) Methyl isopropylether (B.P. 32° C.)
- (4) Dimethyl ether of diethylene glycol (B.P. 162.0° C.)

These ethers are identified by number in Table III.  $\text{CO}_2$  and  $\text{O}_2$  are added for ten minutes at the rate of about 1 g./min. at just above the temperature at which the wax products melt.

Where the products of Part I are further hydrogenated with a compound containing an active hydrogen (see

HYDROGENATION

We have also found that the alkali metal treated wax (or ether-alkali metal treated wax) can be further treated to remove additional trace amounts of undesirable impurities by reacting the wax with either (1) hydrogen or (2) a compound containing an active hydrogen atom.

Thus, the term, "hydrogenation" includes reduction by means of either (1) or (2).

(1) *Hydrogenation with hydrogen of the alkali metal treated wax.*—Hydrogenation is effected by contacting the alkali metal treated wax in a liquid form with hydrogen at elevated temperatures and pressures, the duration of the treatment and the temperature being regulated so that the wax suffers substantially no cracking or splitting into low molecular liquid products.

Any of the conventional systems of hydrogenating hydrocarbons can be employed. For example, temperatures in excess of about 60° C. such as 60 to 300°, for example 80 to 250° but preferably 150 to 200°; at pressures in excess of 10 p.s.i. such as 10 to 500 p.s.i. for example 50 to 450 p.s.i. but preferably 200 to 400 p.s.i. The duration of the treatment will vary depending on conditions such as temperature, pressure, catalyst, etc. However, in general the duration of treatment is generally in excess of 1 min., such as 5 min. to 24 hours, for example 5.0 to 120 min., but preferably 15 to 60 min. The duration of the treatment is generally shortened as the temperature is increased in order to avoid substantial cracking of the wax. Of course, it should be realized that the above conditions are generally stated and can be varied since the conditions are interdependent.

The following are examples of catalyst systems that can be employed in the process:

TABLE IV

| No.  | Catalyst                                                          | Manufacturer                                |
|------|-------------------------------------------------------------------|---------------------------------------------|
| (1)  | 72% Ni on kieselguhr                                              | Harshaw Chemical Company.                   |
| (2)  | 0.5% Pd on alumina                                                | Bohen & Company.                            |
| (3)  | 0.8% Pt, 0.3 Cl, 0.3 F on alumina                                 | Universal Oil Products.                     |
| (4)  | 5% Pt on carbon                                                   | Engelhard Industries.                       |
| (5)  | 10% Ni as nickel oxide on alumina                                 | Harshaw Chemical Company.                   |
| (6)  | 82% $\text{CuO}$ , 17% $\text{Cr}_2\text{O}_3$                    | Do.                                         |
| (7)  | 41% $\text{CuO}$ , 44% $\text{Cr}_2\text{O}_3$ , 11% $\text{BaO}$ | Do.                                         |
| (8)  | Raney Nickel                                                      | W. R. Grace.                                |
| (9)  | Copper-chromium oxide                                             | Prepared according to JACS 72, 2626 (1950). |
| (10) | 5% rhodium on alumina                                             | Engelhard Industries.                       |
| (11) | 5% ruthenium on alumina                                           | Do.                                         |
| (12) | 5% rhodium on carbon                                              | Do.                                         |
| (13) | 5% ruthenium on carbon                                            | Do.                                         |
| (14) | Pd on strontium carbonate                                         | Prepared according to JACS 78, 6299 (1956). |
| (15) | 5% Pd on carbon                                                   | Engelhard Industries.                       |
| (16) | Adam's Catalyst ( $\text{PtO}_2$ )                                | Prepared according to JACS 44, 1397 (1922). |

The above catalysts are merely exemplary of those that can be employed.

Hydrogenation catalysts and processes of hydrogenation are so well known to the art that further examples are unnecessary. The preferred hydrogenation catalysts which are employed are those capable of hydrogenating aromatic compounds. Examples of such catalysts can be found in chapter 4 of *Catalysis*, volume V, Emmett, Reinhold Publishing Corporation (1957) and elsewhere.

The process of hydrogenation can be conducted on a batch or continuous basis using any type of reaction or series of reactions known to the art.

The catalysts may be employed in the form of powder intimately mixed with wax prior to treatment with hydrogen under pressure and at the end of this treatment they are separated from the wax, for example, by filtering, or centrifuging the product and are available for the refining

175-200 p.s.i. for one-half hour. The product is then filtered.

*Example 4*

5 The product of Table II, Ex. 3, Part I, and 1% by weight of ruthenium on alumina are placed in a rocker autoclave and treated with hydrogen at 200-210° C. and 350-400 p.s.i. for one-half hour. The product is then filtered.

10 Other products also hydrogenated are presented in the following table. The designation employed for the product hydrogenated refers to the table, example, and part. Thus II 1, Part I refers to Table II, Example 1, Part I. The catalyst number refers to those catalysts of Table IV. Thus, catalyst 1 refers to 72% Ni on kieselguhr. In all cases the product hydrogenated whether in Part I, II or III is filtered prior to hydrogenation.

TABLE V.—HYDROGENATION WITH H<sub>2</sub>

| Ex. | Product Hydrogenated | Catalyst |                | Time (Hr.) | Temp., °C. | Pressure, p.s.i. |
|-----|----------------------|----------|----------------|------------|------------|------------------|
|     |                      | No.      | Weight percent |            |            |                  |
| 1   | II 1 Part I          | 1        | 1              | 1          | 200-210    | 450-500          |
| 2   | II 1 Part II         | 8        | 1              | 1          | 150-160    | 250-300          |
| 3   | II 1 Part III        | 12       | 1              | 0.5        | 90-100     | 175-200          |
| 4   | II 3 Part I          | 11       | 1              | 0.5        | 200-210    | 350-400          |
| 5   | II 5 Part II         | 15       | 1              | 1          | 60-70      | 175-200          |
| 6   | II 9 Part II         | 4        | 1              | 1          | 100-110    | 225-250          |
| 7   | II 13 Part I         | 1        | 1.5            | 0.75       | 150-155    | 175-200          |
| 8   | II 19 Part III       | 12       | 1              | 1          | 170-175    | 200-225          |
| 9   | II 2 Part I          | 11       | 1              | 1          | 200-215    | 210-240          |
| 10  | III 1 Part I         | 15       | 0.5            | 1.5        | 140-150    | 275-300          |
| 11  | III 1 Part II        | 4        | 0.5            | 1.5        | 120-125    | 300-325          |
| 12  | III 4 Part II        | 1        | 0.05           | 2          | 145-155    | 225-250          |
| 13  | III 6 Part I         | 12       | 0.5            | 1.5        | 190-200    | 275-300          |
| 14  | III 8 Part II        | 1        | 0.05           | 1.75       | 200-215    | 375-400          |
| 15  | III 10 Part I        | 4        | 0.5            | 1.5        | 190-200    | 150-175          |
| 16  | III 12 Part III      | 11       | 1              | 1          | 140-150    | 175-200          |
| 17  | III 13 Part I        | 1        | 1              | 1          | 170-175    | 175-200          |

of additional wax. The catalysts may, however, be disposed separately, in a coarse form in the reaction chamber the molten wax being then passed over them with a counter- or equidirectional flow of hydrogen. For example, a mixture of melted wax and hydrogen gas is fed to the hydrogenation reaction containing the catalyst. This mixture is preferably preheated to the reaction temperature and the reaction is maintained at the desired pressure during the passage of the melted wax therethrough. Unconsumed hydrogen is separated from the products and may be recycled through the hydrogenation reaction.

As previously noted herein, before hydrogenation it is desirable to filter the alkali metal treated wax since the precipitate tends to inactivate the hydrogenation catalyst.

TABLE V EXAMPLES

*Example 1*

The filtered product of Table II, Ex. 1, Part I, is placed on rocker autoclave and 1% by weight of nickel catalyst (on kieselguhr) is added thereto. The system is swept with hydrogen and then pressurized. The temperature is then raised to 200-210° C. for 1 hour at an operating pressure of 450-500 p.s.i. The product is then filtered.

*Example 2*

The filtered product of Table II, Ex. 1, Part II, and 1% by weight of Raney nickel are charged to a rocker autoclave. The system is swept with hydrogen, heated to 150-160° C. at 250-300 p.s.i. and thus maintained for one hour. The product is then centrifuged.

*Example 3*

The filtered product of Table II, Ex. 1, Part III, and 1% by weight of rhodium on carbon are placed in a rocker autoclave and treated with hydrogen at 90-100° C. and

40 (2) *Reaction of the alkali metal treated wax with a compound containing an active hydrogen.*—In general, compounds containing an active hydrogen can be substituted for hydrogen in hydrogenation only in the case of the alkali metal treated wax that has not been carbonated or oxygenated. This is in contrast to hydrogenation with hydrogen which can be employed in all instances, including the carbonated and oxygenated product.

In general, at least one

50  $\text{gram-mol}$   
No. of active hydrogen on molecule

of the active hydrogen compound is added for each gram-atom of alkali metal.

55 In practice, however, excesses of active hydrogen compounds are employed for example 5-10% or more of the active hydrogen compound based on weight of wax.

60 As previously noted, after filtration of the alkali metal-treated wax it is advisable to examine the wax filtrate for condensed ring aromaticity. If the wax filtrate tests positively for condensed ring aromaticity, one adds additional alkali metal, preferably with ether, and then proceeds to hydrogenate with an active hydrogen compound in the manner of this invention.

65 By a "compound containing an active hydrogen" we mean a compound having an active hydrogen which is capable of reacting with an alkali metal or an alkali metal organic compound, for example, the reaction product of sodium and a condensed ring aromatic compound.

The addition of compounds containing an active hydrogen to alkali metal treated wax results in a wax containing less impurities. Examples of such compounds comprise alcohols, for example methanol, ethanol, propanol, etc., acids, for example formic, acetic, propionic, etc. acids and the like.

In carrying out the process, these compounds are added to the alkali metal treated wax so as to react with the components present therein at a temperature sufficient to cause reaction, the duration of the treatment and the temperature being regulated so that the wax suffers substantially no cracking or splitting into low molecular liquid products such as occurs at temperatures in excess of 300° C., for example 60° to 200° C., but preferably 60 to 150° C.; for a period of at least 1.0 min. such as 1.0 to 120 min., for example 5 to 90 min., but preferably 10 to 30 min. Whenever convenient, it is preferred to run the reaction at reflux. The conditions of the treatment will vary depending on the compound employed. The duration of the treatment is generally shortened as the temperature is increased in order to avoid substantial cracking of the wax. Where the compound containing an active hydrogen is low boiling, superatmospheric pressure can be employed. Excess amounts of the compound after reaction can then be removed under reduced pressure.

TABLE VI EXAMPLES

## Example 1

The product of Table II, Ex. 1, Part I (unfiltered), and 10% by weight of methanol are heated at reflux for 20 minutes. The product is then filtered. Excess methanol is distilled from the product.

## Example 4

The product of Table II, Ex. 8, Part I (unfiltered), and 10% by weight of ethanol are heated at reflux for 15 minutes. The product is then filtered. Excess ethanol is distilled from the product.

## Example 6

The product of Table II, Ex. 13, Part I (unfiltered), and 10% by weight of acetic acid are heated at reflux for 15 minutes. The product is then filtered. Excess acetic acid is distilled from the product.

The following examples are carried out in a similar manner. Ten percent (by weight based on wax) of the active hydrogen compounds is employed in all examples and the reaction mixture heated to reflux. Where ether is employed in the prior step, the alkali metal ether treated product is not freed from ether until after treatment with a compound containing an active hydrogen and prior to filtration.

TABLE VI.—HYDROGENATION WITH COMPOUNDS HAVING ACTIVE HYDROGENS

| Ex. | Product Treated | Active Hydrogen Compound, Name | Time (Min.) |
|-----|-----------------|--------------------------------|-------------|
| 1   | II 1 Part I.    | Methanol.....                  | 20          |
| 2   | II 2 Part I.    | do.....                        | 10          |
| 3   | II 5 Part I.    | do.....                        | 20          |
| 4   | II 8 Part I.    | Ethanol.....                   | 15          |
| 5   | II 10 Part I.   | Propanol.....                  | 20          |
| 6   | II 13 Part I.   | Acetic acid.....               | 15          |
| 7   | II 14 Part I.   | do.....                        | 15          |
| 8   | II 17 Part I.   | Formic acid.....               | 15          |
| 9   | II 21 Part I.   | Propionic acid.....            | 20          |
| 10  | III 1 Part I.   | Formic acid.....               | 20          |
| 11  | III 2 Part I.   | Propanol.....                  | 20          |
| 12  | III 3 Part I.   | Methanol.....                  | 10          |
| 13  | III 4 Part I.   | Ethanol.....                   | 10          |
| 14  | III 7 Part I.   | do.....                        | 10          |
| 15  | III 10 Part I.  | do.....                        | 10          |
| 16  | III 13 Part I.  | Acetic acid.....               | 10          |
| 17  | III 14 Part I.  | do.....                        | 15          |

## FURTHER TREATMENT OF WAX FILTRATE III PRODUCT

The following examples are presented to illustrate further treatment of the product of alkali metal treated wax, after precipitate removal (i.e. wax filtrate III).

## Example A

Example A1.—Wax filtrate III obtained from Table II, Example 1, Part I, is found to contain condensed ring

aromaticity. Thereupon, 0.5% sodium and 1,2-dimethoxyethane is added in an ether to wax ratio of 0.25 and heated to reflux for one hour. The resulting product is divided into Part I, Part II, and Part III.

- 5     Example A2.—Part I is blown with CO for ten minutes, ether is distilled from the wax, and the precipitate formed removed by filtration. The product has no measurable condensed ring aromaticity as measured by ultra-violet absorbence and fluorescence. The product is AI wax.
- 10    Example A3.—Part II is blown with O<sub>2</sub> for ten minutes, ether is distilled from the wax, and the precipitate formed removed by filtration. The product contains measurable condensed ring aromaticity as determined by ultra-violet absorbence and fluorescence. The product is a DI wax.
- 15    Example A4.—This product is then hydrogenated with hydrogen for one hour at 200–210° C. and 450–500 p.s.i. in the presence of 1% Ni (72%) on kieselguhr. After treatment no measurable condensed ring aromaticity is observed. The product is a DII wax.
- 20    Example A5.—Part III is heated with 10% by weight of ethanol at reflux for 15 min., excess ether and alcohol are distilled from the wax, and the precipitate then removed by filtration. The product formed has no measurable condensed ring aromaticity. The product is an EI wax.

## Example B

Wax filtrate III from Table II, Ex. 5, Part I, treated with Na-K 50:50 alloy is found to contain very low condensed ring aromaticity when tested by ultra-violet absorbence.

- 30    Similar treatment can be effected with other wax filtrates III products formed in accordance with this invention, for example those of Table II, Part I.
- 35    The waxes refined by the processes of this invention either by alkali metal alone, or by alkali metal ether, or either of these processes in combination with hydrogenation, oxygenation, carbonylation, or oxygenation followed by hydrogenation, or carbonylation followed by hydrogenation, carbonylation followed by hydrogenation, etc., are characterized by the removal of or the reduction in color and color-forming bodies, aromatic content, sulfur, nitrogen, combined oxygen, trace metals and other undesirable materials.
- 40    45    Besides producing a wax of excellent physical properties such as in regard to melting point, plasticity, penetration, etc., an additional advantage of these processes over other refining processes is that they present a facile method of removing color and color-forming bodies and other impurities which are either too difficult or too expensive to remove by other methods. They are particularly effective in removing condensed ring aromaticity present in the wax. Convenient and acceptable methods which we have employed in determining the amount of condensed ring aromaticity in waxes comprises subjecting wax to an ultra-violet and/or fluorescent examination. Based on such examination the condensed ring aromaticity of alkali metal treated waxes is less than the condensed ring aromaticity of the wax prior to treatment. However, the condensed ring aromaticity of wax subjected to alkali metal alone (although substantially reduced from the wax prior to treatment) is not as much reduced as when the wax is treated with alkali metal in combination with oxygenation, carbonation, or hydrogenation, or combinations thereof.

Aromaticity, especially in terms of condensed ring aromaticity, can be effectively determined by both ultra-violet absorption spectra and fluorescence spectra. The spectra obtained allows qualitative and quantitative determination to be made on the wax or any component removed from the wax, by such means as chromatography. Condensed ring aromatics exhibit characteristic spectra of both types which are characteristic of their structure, so that matching with spectra of known compounds is

practical. This type of analysis lends itself readily to the determination of extremely low concentrations (in the order of ten parts per billion) as has been illustrated in the literature.

In general, ultraviolet absorption spectra are obtained by the following procedure:

A 1-3% solution of the wax is prepared using spectroscopically pure iso-octane. The concentration may be adjusted in some cases if too large or too small of an amount of absorbing material is present in the wax. Quartz cells are used and the wax solution is run against the solvent used. Any ultraviolet spectrophotometer may be used if the spectra between 260-330 millimicrons can be scanned using a hydrogen lamp as the light source. Any components separated from the wax by chromatographic procedures, distillation, extraction, etc., can be analyzed using this same general procedure. The procedure published by Lizinsky, W., *Analytical Chemistry*, 32, 684-687 (1960) is illustrative.

In general, fluorescent spectra are obtained by the following procedure:

Solid samples of wax either in quartz cells or as solid plates of wax are employed. Any fluorometer or ultraviolet spectrophotometer with fluorometer attachment, such as available for the Beckman DK-1 or DU instruments, is suitable. The procedure as outlined by Eichkoff, H. J., and Tischack, G., Erdol und Kohle 705-708 (1958) is generally used. Also, as with the ultraviolet spectra, any components that can be isolated by chromatographic procedures, distillation, etc., can be examined using a solution with a solvent, such as spectroscopically pure iso-octane or ethanol.

In both cases, i.e., with ultraviolet and fluorescent examination, qualitative and quantitative determinations are made by comparing the spectra of the unknown wax with that known compounds or by comparing the spectra of the unknown wax with the spectra of components separated from the wax.

Although various embodiments of our invention have been described herein, many variations thereof can be practiced without departing from the spirit of the invention.

For example, any of the procedures described herein in the specification and claims can be practiced in conjunction with conventional wax refining techniques such as treatment with absorbent materials such as bauxite, clay, alumina, charcoal, silica gel and the like. Such treatment can be carried out as a step in the process or subsequent to the completion of the process.

In addition to the alkali metals described herein, certain alkali metal compounds which react in the manner of alkali metals can also be employed, for example, alkali metal alkyls such as ethyl sodium, alkali metal-alkali earth alloys for example the sodium-calcium alloys, alkali metal-ammonia combinations, alkali metal-amine combinations, sodamide, etc.

In all cases except carbonated or oxygenated wax, the term "hydrogenating" as employed herein refers to treating the wax with either hydrogen or a compound containing an active hydrogen. With carbonated or oxygenated wax, the term "hydrogenation" refers only to hydrogenation with hydrogen.

The term, "hydrocarbon wax" as employed herein refers the wax itself or wax-containing composition such as intermediates in the preparation of hydrocarbon waxes.

These waxes are particularly useful in food applications, such as food wrappers, food cartons, etc.

Having thus described our invention, what we claim as new and desire to obtain by Letters Patent is:

1. A process of refining a hydrocarbon wax which includes treating said wax first with an alkali metal alone and then hydrogenating said wax.

2. A process of refining a hydrocarbon wax which includes treating said wax with an alkali metal alone in the presence of a stable ether selected from the group consisting of (1) an aliphatic ether containing a  $\text{CH}_3\text{O}$ -group and (2) a cyclic aliphatic ether, a number of oxygen atoms and the number of carbon atoms in said stable ether being in a ratio of not less than 1:4, and then hydrogenating said wax.

3. A process of refining a hydrocarbon wax which includes treating said wax first with an alkali metal alone, separating the wax from the precipitate formed, then hydrogenating said wax, and then separating the wax from the precipitate formed.

4. A process of refining a hydrocarbon wax which includes treating said wax with an alkali metal alone in the presence of a stable ether selected from the group consisting of (1) an aliphatic ether containing a  $\text{CH}_3\text{O}$ -group and (2) a cyclic aliphatic ether, the number of oxygen atoms and the number of carbon atoms in said stable ether being in a ratio of not less than 1:4, removing said ether, separating the wax from the precipitate formed, hydrogenating said wax and then separating the wax from the precipitate formed.

5. A process of refining a hydrocarbon wax, which has been treated with an alkali metal alone in the absence of ether and then separated from the precipitate formed, which includes hydrogenation of said treated and separated wax with hydrogen.

6. A process of refining a hydrocarbon wax, which has been treated with alkali metal alone in the absence of ether and then separated from the precipitate formed, which includes further treatment of said treated and separated wax with alkali metal in the presence of an ether selected from the group consisting of (1) an aliphatic ether having a  $\text{CH}_3\text{O}$ -group and (2) a cyclic aliphatic ether, the number of oxygen atoms and the number of carbon atoms in the stable ether being in the ratio of not less than 1:4, and then hydrogenating the product with a compound having an active hydrogen.

#### References Cited by the Examiner

##### UNITED STATES PATENTS

|           |         |                 |         |
|-----------|---------|-----------------|---------|
| 1,983,220 | 12/1934 | Fields          | 208-284 |
| 2,042,557 | 6/1936  | Sparks          | 208-294 |
| 2,385,431 | 9/1945  | Vose            | 208-284 |
| 2,586,198 | 2/1952  | Backlund et al. | 208-27  |
| 2,789,134 | 4/1957  | Nelson et al.   | 208-284 |
| 2,908,702 | 10/1959 | Haines et al.   | 208-20  |
| 2,915,448 | 12/1959 | Annable et al.  | 208-27  |
| 2,956,001 | 10/1960 | Spars et al.    | 208-27  |
| 3,056,773 | 10/1962 | Joo et al.      | 208-294 |

##### FOREIGN PATENTS

|         |        |          |
|---------|--------|----------|
| 247,357 | 5/1912 | Germany. |
|---------|--------|----------|

##### OTHER REFERENCES

Dietz et al.: *Ind. & Eng. Chem.*, vol. 44, No. 8, August 1952, pages 1818, and 1819.

65 DELBERT E. GANTZ, *Primary Examiner*.

ALPHONSO D. SULLIVAN, *Examiner*.

H. LEVINE, *Assistant Examiner*.